

## UNITED STATES PATENT OFFICE

2,200,088

## ELECTRICAL CONTACT MEMBER

James M. Kelly, Trafford, Pa., assignor to Westinghouse Electric & Manufacturing Company, East Pittsburgh, Pa., a corporation of Pennsylvania

No Drawing. Application September 14, 1938,  
Serial No. 229,866

9 Claims. (Cl. 200—166)

This invention relates to electrical make and break contact members.

Contact members of refractory metal powders and a metal having good conductivity such as 5 copper or silver have been employed heretofore. Recently carbon has been so added to the composition of the contact members that when heat treated it will combine with the refractory metal and form a refractory carbide, thereby increasing 10 the hardness of the contact member. Such refractory carbide is undesirable since it increases the resistivity of the metal and lowers the melting point of the refractory with which it combines.

15 An object of this invention is to provide a contact member having high physical properties, wear characteristics and good conductivity.

Another object of this invention is to provide a composite contact member formed from refractory metal powders and an alloy of copper, 20 cobalt and iron.

A further object of this invention is to provide a contact member formed from refractory metal powders and an alloy which is susceptible to an 25 age hardening heat treatment to give high physical properties and good conductivity to the contact member.

Other objects of this invention will become apparent from the following description and the 30 appended claims.

In practicing the present invention, a contact member is formed from a plurality of metals which have been found to cooperate to give certain desired characteristics. A base body of refractory metal selected from the group tungsten, 35 molybdenum and tantalum and which has a relatively high melting point so formed as to have interstices therein and which of itself does not possess the desired characteristics is impregnated 40 with a copper base alloy of lower melting point as will be disclosed more fully hereinafter to give a resulting product having the desired characteristics.

In forming the metal base here employed, refractory metal powders of a predetermined size 45 ranging from 150 to 250 mesh are formed into a slug of a suitable size and shape. The metal refractory powder can be compressed in a steel die under pressures ranging from 5 to 15 tons per 50 square inch depending upon the amount of voids or the porous structure it is desired to produce in the body or base after which it is impregnated with the alloy utilized in this invention.

Another way of forming the refractory metal 55 base is to mix the refractory metal powders of

predetermined size with sufficient organic bond to form a plastic putty-like mass which is moldable or which may be rolled and cast to a desired shape. Any suitable organic bond which can be removed by drying or sintering the shaped 5 mass to leave a porous structure may be employed. It is highly desirable to employ a bond which can be substantially completely removed so as not to leave a carbon residue which may combine with the refractory metal in the form of 10 a carbide since such carbides are undesirable. An organic bond composed of about 75% of shellac and 25% of alcohol is entirely satisfactory in forming the putty-like mass, and when the mass is heated at a temperature of about 1000° C. in a 15 reducing atmosphere, is substantially completely removed leaving the desired porous base of refractory metal.

In order to impart the desired electrical characteristics to the contact member, the porous 20 refractory metal base or slug is then filled with the impregnating alloy. The alloy employed in the contact member of this invention is a copper base alloy which contains cobalt and iron as essential elements therein in predetermined proportions as disclosed and claimed in James M. Kelly's copending application Serial No. 149,146, filed June 19, 1937, now Patent 2,147,844 and directed to Copper base alloys.

In the impregnating alloy, the cobalt and iron 25 are each present in amounts ranging from a small but effective amount up to 5% with the balance substantially all copper. As disclosed in the hereinbefore identified Kelly Patent, a preferred range of each of the cobalt and iron contents is 30 between .5% to 3% while the best combination of properties are obtained where the ratio of the cobalt to iron in the alloy is between .5 and 1.25 to 1 with a preferred ratio of 1 to 1. These alloys are susceptible to age hardening and when 35 treated as by quenching them from a temperature of between 750° C. and 1075° C. and aged at a temperature between 450° C. and 600° C. have an 40 electrical conductivity of 60% or greater, and a hardness approximating 80 Rockwell B or 45 greater.

When the slug or body of the contact member is so formed from the refractory metal powders in either of the ways described hereinbefore as to have a predetermined porosity, it is impregnated 50 with the copper-cobalt-iron alloy. In practice the refractory metal powders may be so formed that the body will comprise from 50% to 90% of the finished contact member, the balance being the copper base alloy having the cobalt 55

and iron present in the quantities and ratios indicated hereinbefore. With the organic bond method of making the refractory metal body, it is possible to secure a more uniform and more porous body, so that when it is desired to employ an alloy content of from 30% to 40% in the contact member the organic bond method of forming the refractory metal body is preferably utilized.

10 In order to impregnate the refractory metal body or base of the contact member, the pre-formed base is placed in a suitable furnace in a refractory container in the presence of a definite amount of the copper-cobalt-iron alloy and subjected to heat at a temperature above the melting point of the alloy, but below the melting point of the refractory metal in a reducing atmosphere. At this temperature the alloy melts, wets and impregnates the porous refractory base securely bonding to the refractory to form a strong homogeneous article when cooled.

20 For general applications, contact members of from 80% to 55% of the refractory metal powders impregnated with from 20% to 45% of the copper base alloy having a cobalt content of from .5% to 3% and an iron content of from .5% to 3% and in which the cobalt to iron ratio is between .5 and 1.25 to 1 are satisfactory.

30 Where the organic bond method is employed in making the refractory metal base, it is found that the resulting impregnated contact member responds to a heat treatment as described hereinbefore for effecting the age hardening of the copper base alloy in the contact member to improve the physical and electrical characteristics of the contact member over those characteristics obtained in the unheat treated contact members. However, when the refractory metal base is formed by the pressure method, it is found that 40 a heat treatment to age harden the impregnating alloy is not always necessary unless it is desired to improve the conductivity, since the copper base alloy particles in the contact member are so small that hardening them has substantially no effect 45 on increasing the hardness of the contact member as a unit. Even without the heat treatment the hardness values obtained in contact members formed under the high pressure method are as a general rule somewhat higher than those obtained in the contact members formed by the organic bond method. In both cases the contact members produced have excellent physical and electrical properties.

50 Contact members of the refractory metal tungsten impregnated with the copper-cobalt-iron alloy and which are representative of the contact members comprising this invention are as follows:

| No. | Percent W | Percent Cu | Percent Co | Percent Fe |
|-----|-----------|------------|------------|------------|
| 10  | 76.48     | 22.40      | .5         | .59        |
| 20  | 60.54     | 37.68      | .86        | 1.01       |
| 30  | 60.00     | 38.95      | .48        | .57        |

65 In making the contact member No. 10, the tungsten powders of 200 mesh size were compacted into the predetermined shape of the base of the contact member under 15 tons pressure while the organic bond method was employed in making contact members Nos. 20 and 30 utilizing tungsten powders of the same size. All of the contact members have hardness values of 80 Rockwell B or better, some ranging as high 75 as 108. The age hardening heat treatment indi-

cated hereinbefore increases the hardness and conductivity of the contact members over the values obtained in the untreated contact members formed by the organic bond method and improves the conductivity of the contact members 5 formed by the pressure method.

Under test conditions, the contact members of this invention consistently have a life of more than 119,000 operations or interruptions when employed as the contact members in an oil circuit breaker connected in a three-phase circuit and operated under rated conditions of 60 amperes, 440 volts at 60 cycles, with reactors connected in the circuit to serve as the load and to provide a low power factor. In the test the breaker was tripped at the rate of 27 times per minute for measuring the life of the contact members.

By practicing this invention, contact members are produced having an extremely high hardness 20 and good conductivity which are free from the carbon contamination employed heretofore for improving the wear characteristics of the contact members. The alloy employed in the contact members imparts the desired characteristics, 25 both physical and electrical, which are desired in the contact member, providing a contact member having wear resistance, low resistivity and good conductivity. Further such contact members can be brazed to the contactor arm to give a 30 good rigid electrical connection without detrimentally affecting the physical and electrical characteristics of the contact member.

Since certain changes may be made in the processes described hereinbefore, and certain modifications may be made in the resulting disclosed contact member which embodies the invention without departing from its scope, it is intended that all matter contained in the above description shall be interpreted as illustrative and not 40 in a limiting sense. This invention is therefore not to be limited except insofar as is necessary in accordance with the teachings of the prior art and the scope of the appended claims.

I claim as my invention:

1. An electrical contact member comprising a body portion of refractory metal powders bonded together with an alloy comprising from .5% to 5% of cobalt, from .5% to 5% of iron with the balance substantially all copper.

2. An electrical contact member comprising from about 90% to 50% of refractory metal powders and from about 10% to 50% of a copper, cobalt and iron alloy, the alloy comprising from .5% to 5% of cobalt and from .5% to 5% of iron with the balance substantially all copper.

3. An electrical contact member comprising from 80% to 50% of refractory metal powders impregnated and integrally united with from 20% to 50% of an alloy composed of from .5% to 3% of cobalt, from .5% to 3% of iron with the balance copper.

4. An electrical contact member comprising from 80% to 50% of refractory metal powders impregnated and integrally united with from 20% to 50% of an alloy composed of from .5% to 3% of cobalt, from .5% to 3% of iron with the balance copper, the impregnated refractory metal being heat treated to give high physical strength and conductivity to the alloy.

5. An electrical contact member comprising from 80% to 55% of tungsten powders formed to a predetermined shape and impregnated with from 20% to 45% of an alloy composed of from .5% to 3% of cobalt, .5% to 3% of iron with 75

the balance copper and in which the ratio of the cobalt to the iron content is between .5 and 1.25 to 1.

6. An electrical contact member as in claim 2  
5 which has been quenched from a temperature of between 750° C. and 1075° C. and aged at a temperature of between 450° C. and 600° C.

7. An electrical contact member comprising about 76.5% of tungsten powders, about 22.4%  
10 of copper, about .5% of cobalt and about .6% of iron, the copper, cobalt and iron being in the form of an alloy bonding the tungsten powders.

8. An electrical contact member comprising about 60.5% of tungsten, about 37.7% of copper, about .85% of cobalt and about 1% of iron, the copper, cobalt and iron being in the form of an alloy bonding the tungsten powders. 6

9. An electrical contact member composed of about 60% by weight of tungsten and 40% by weight of an alloy having the analysis of 1.45% of iron and 1.20% of cobalt with the balance copper. 10

JAMES M. KELLY.